

Sept. 16, 1958

H. ULRICH ET AL

2,852,374

PHOTOGRAPHIC DEVELOPER

Filed March 16, 1955



INVENTORS:

HANS ULRICH, RUDOLF MERSCH, OTTMAR WAHL, DETLEF DELFS.  
BY

*Connolly and*  
*their ATTORNEYS*

## PHOTOGRAPHIC DEVELOPER

Hans Ulrich, Köln-Stammheim, Rudolf Mersch, Leverkusen-Bayerwerk, and Ottmar Wahl and Detlef Delfs, Opladen, Germany, assignors to AGFA Aktiengesellschaft für Photofabrikation, Leverkusen, Germany, a corporation of Germany

Application March 16, 1955, Serial No. 494,687

Claims priority, application Germany March 18, 1954

11 Claims. (Cl. 96—66)

The present invention relates to photographic silver halide developing substances and especially to such substances which are derived from 1-phenyl-3-amino-pyrazolines.

1-phenyl-3-amino-pyrazoline has only a very slight activity as a photographic developer, so that it is of no practical value. The same also applies for its sulpho acid or carboxylic acid derivatives which are readily soluble in alkali. Moreover, the substitution of the aryl radical by aliphatic substituents does not provide any substantial change as regards the developing power.

It has now been found that 1-aryl-3-amino-pyrazolines, which contain OH or NH<sub>2</sub> groups as substituents in the aryl radical in the 4-position are highly active developers with very valuable photographic properties, it being possible for the hydrogen atoms of the NH<sub>2</sub> group to be replaced by organic radicals as for instance by alkyl, oxalkyl, sulpho-alkyl or carboxy-alkyl groups. If necessary, the aryl radical may also carry other substituents apart from OH or NH<sub>2</sub> groups, such as alkyl groups and halogen atoms.

Such compounds are not only very rapidly acting photographic developers when used alone in alkaline solution, but they show super-additive effects to a degree not hitherto known, particularly in combination with known types of silver halide developing substances, such as pyrocatechol, pyrogallol, hydroquinone, p-aminophenol, o-aminophenol, o- and p-aminophenols substituted in the aromatic nucleus or in the amino group, such as p-methylaminophenol and N-p-oxyphenylglycin, 2,4-diaminophenol, o- and p-phenylenediamin and derivatives thereof. As an additive to less active developers, they have such a strong activating effect even in minimum amounts that completely novel effects may be produced. As is known, the combinations of hydroquinone and p-methylaminophenol are the standard developers which are most commonly used because of their valuable properties. If the p-methylaminophenol in such standard developers is replaced by a few percent by weight of the novel compounds, not only is it possible to obtain development effects which are comparable to the hydroquinone-p-methylaminophenol developer, but there may additionally be produced substantially more advantageous effects. Such developers, for example, become operative more quickly, they provide higher threshold values and steeper gradation with deeper blackening. The special action of the developer substances is also obtained, if they are present for instance in developing solutions which are used for developing silver halide layers, which contain known developing substances. Furthermore the developing substances according to the present invention may be incorporated into silver halide layers by themselves or in combination with other known developing substances, whereafter these layers are developed either in alkaline aqueous solution or in alkaline aqueous solution containing developing substances.

Despite the very small amount which is used as compared with p-methylaminophenol, for example  $\frac{1}{20}$  to

$\frac{1}{50}$  of the usual p-methylaminophenol quantities, such developers are of high strength, in that an almost complete regeneration of the activator takes place by exchange action with the hydroquinone, so that it is possible to refer to a catalytic action of the novel compounds. These developer mixtures are, therefore, characterized by being particularly inexpensive. Furthermore, it is possible therewith to produce special developers for a wide variety of purposes in the photographic art.

The said 1-aryl-3-aminopyrazolines may be obtained by the processes disclosed in British patent specification 679,678 or by the processes of the co-pending application Ser. Nos. 440,562, now abandoned, assigned to the same assignee as the present application. As starting materials there may for instance be used  $\beta$ -N-aryl-N-nitroso-aminopropionic acid nitriles, which are suitably substituted in the aryl group, these nitriles being reduced in acid solution, for example with powdered zinc. The  $\beta$ -N-aryl-N-nitroso-aminopropionitriles serving as initial material for this process are readily obtainable by nitrosoing  $\beta$ -aryl-aminopropionitriles which in turn are available by reaction of aromatic amines with aryl nitrile. The above reaction is illustrated by the following equation:



In the following examples, the parts which are indicated are parts by weight:

### Example I

A grey step wedge (factor  $f = \sqrt[3]{2}$ ) is exposed on normal silver chloride paper ("Agfa Lupex") of normal gradation on a sensitometer. The development is carried out at 20° C. in solutions of the following composition:

|                                         | A     | B     | C     | D     | E     | F     |
|-----------------------------------------|-------|-------|-------|-------|-------|-------|
| Water                                   | 1,000 | 1,000 | 1,000 | 1,000 | 1,000 | 1,000 |
| Hydroquinone                            | 3     | 3     | 3     | 3     | 3     | 3     |
| Na-sulphite anhyd.                      | 13    | 13    | 13    | 13    | 13    | 13    |
| Soda anhyd.                             | 26    | 26    | 26    | 26    | 26    | 26    |
| Potassium bromide                       | 1     | 1     | 1     | 1     | 1     | 1     |
| p-methylaminophenol                     | 1     |       |       | 0.05  |       |       |
| 1-(p-hydroxy-phenyl)-3-amino-pyrazoline |       | 0.05  |       |       |       |       |
| 1-phenyl-3-hydroxypyrazoline            |       |       | 0.05  |       |       |       |
| 1-phenyl-3-amino-pyrazoline             |       |       |       |       |       | 0.05  |

The first image traces appear with

- Developer A after 11 seconds
- Developer B after 11 seconds
- Developer C after 15 seconds
- Developer D after 35 seconds
- Developer E after 50 seconds
- Developer F after 50 seconds

After one minute, the development is stopped by a 2% acetic acid bath and fixed in the normal manner. A comparison of the points shows the following:

As compared with Developer A

- Developer B shows one grey step more,
- Developer C shows one grey step less,
- Developer D shows eight grey steps more,
- Developer E shows only a flat image trace,
- Developer F shows only a flat image trace.

Developer B, therefore, gives the deepest blackening.

**3**  
**Example 2**

Grey step wedges are exposed as in Example 1 on silver chloride or silver bromide papers and developed in developers of the following composition:

|                                        | A     | B     | C     |
|----------------------------------------|-------|-------|-------|
| Water                                  | 1,000 | 1,000 | 1,000 |
| Hydroquinone                           | 6     | 6     | 6     |
| Na <sub>2</sub> SO <sub>3</sub> anhyd. | 40    | 40    | 40    |
| Na <sub>2</sub> CO <sub>3</sub> anhyd. | 40    | 40    | 40    |
| KBr                                    | 1.5   | 1.5   | 1.5   |
| p-Methylaminophenol                    | 2.5   |       |       |
| 1-(p-hydroxyphenyl)-3-aminopyrazoline  |       | 0.125 |       |
| 1-phenyl-3-hydroxypyrazoline           |       |       | 0.125 |

Using a silver chloride paper, the first traces of the image appear with

Developer A after 6 seconds,  
Developer B after 6 seconds,  
Developer C after 8 seconds,

and when using the silver bromide paper, with

Developer A after 13 seconds,  
Developer B after 10 seconds,  
Developer C after 15 seconds.

After one minute, the development is stopped. The great rapidity of developer B is expressed in an advance of 1½ grey steps as compared with A and C.

If the developers A, B and C are previously exhausted in similar manner by development of 3 square metres of silver bromide paper per litre of developer, then 2 to 3 grey steps more are visible with developer B than with developers A and C.

This ratio is not changed in any way if the developer is subjected to the action of air in such manner that a moderate current of air is drawn in for twenty hours in gas-washing bottles.

In all cases developer B shows the deepest blackening.

**Example 3**

A grey step wedge (factor  $f=2$ ) is exposed on the technical photographic silver halide film "Agfa-Printon R" on a sensitometer. Each is developed for four minutes at 19° C. in the developers of the following composition:

|                                                 | A     | B     | C     | D     | E     | F     |
|-------------------------------------------------|-------|-------|-------|-------|-------|-------|
| Water                                           | 1,000 | 1,000 | 1,000 | 1,000 | 1,000 | 1,000 |
| Na <sub>2</sub> SO <sub>3</sub> anhyd.          | 40    | 40    | 40    | 40    | 40    | 40    |
| Hydroquinone                                    | 6     | 6     | 6     | 6     | 6     | 6     |
| K <sub>2</sub> CO <sub>3</sub>                  | 40    | 40    | 40    | 40    | 40    | 40    |
| KBr                                             | 3     | 3     | 3     | 3     | 3     | 3     |
| p-Methylaminophenol                             | 5     | 0.17  |       |       |       |       |
| 1-(p-hydroxyphenyl)-3-aminopyrazoline           |       |       | 0.17  |       |       |       |
| 1-(p-acetaminophenyl)-3-aminopyrazoline         |       |       |       | 0.17  |       |       |
| 1-(p-N-methylacetaminophenyl)-3-aminopyrazoline |       |       |       |       | 0.17  |       |

From the diagram shown in the accompanying drawing it is readily possible to read off the sequence of the developers as regards their activity. It increases from the developer F in the sequence F, E, D, B, A, C.

**Example 4**

A silver halide layer prepared from a silver halide emulsion containing per litre 7 g. of pyrocatechol is developed after exposure in aqueous solution of sodium hydroxide. If 3 g. of 1-(p-aminophenyl)-3-aminopyrazoline are added to one litre of said solution, the development takes place in a shorter time and leads to a steeper gradation. It is also possible to obtain a similar result by using aqueous solutions of sodium carbonate, which contain per litre 3-5 grams of the aforementioned pyrazolines as for instance 1-(p-methylaminophenyl)-3-aminopyrazoline.

**4**  
**Example 5**

In a developer A for silver chloride and silver bromide papers, of the following composition:

|    |                              |       |      |
|----|------------------------------|-------|------|
| 5  | p-Methylaminophenol-sulphate | grams | 2.5  |
|    | Sodium sulfite               | do    | 40   |
|    | Hydroquinone                 | do    | 6    |
|    | Potassium carbonate          | do    | 40   |
| 10 | Potassium bromide            | do    | 2    |
|    | Benzotriazole                | do    | 0.03 |
|    | Water                        | ml    | 1000 |

the p-methylaminophenol-sulfate is replaced by 0.125 gram of 1-(p-methylaminophenyl)-3-amino-pyrazoline-dihydrochloride or 0.132 gram of 1-(p-ethylaminophenyl)-3-amino-pyrazoline-dihydrochloride (developer B). A third developer C contains only an equimolecular amount, i. e. 0.082 gram, of p-methylaminophenol.

Prints are produced from a negative and developed in the aforesaid developers. The printing process using the developer B takes only 85% of the time of exposure required by developer A. Moreover, development of the image with developer B proceeds at higher velocity than with developer A. The advance in time is about 15%. Developer C works slowly and yields only a flat trace of an image.

The 1-(p-methylaminophenyl)-3-amino-pyrazoline is obtained by refluxing 23.2 grams of 1-(p-acetethylaminophenyl)-3-aminopyrazoline (freezing point F. P. 263° C.) with 270 ml. of 10% aqueous sodium hydroxide solution for 10 hours and cooling the reaction mass, whereby the first mentioned compound crystallizes. It is transformed into the hydrochloride according to customary methods. The 1-(p-ethylaminophenyl)-3-amino-pyrazoline is produced by the same method from 1-(p-acetethylaminophenyl)-3-aminopyrazoline. (F. P. about 140° C. under decomposition.)

**Example 6**

In a developer A for silver chloride and silver bromide papers, of the following composition:

|    |                             |       |      |
|----|-----------------------------|-------|------|
| 30 | p-Methylaminophenol-sulfate | grams | 2.5  |
|    | Sodium sulfite              | do    | 35   |
|    | Hydroquinone                | do    | 6    |
|    | Potassium carbonate         | do    | 40   |
| 35 | Potassium bromide           | do    | 1.5  |
|    | Benzotriazole               | do    | 0.03 |
|    | Water                       | ml    | 1000 |

the p-methylaminophenol-sulfate is replaced by 0.20 gram of the free base 1-(p-aminophenyl)-3-amino-pyrazoline or by 0.28 gram of the corresponding dihydrochloride (=developer B). The developer B is more stable to oxidation by air and of higher capacity than developer A. Thus, for instance a solution containing a given amount of developer B is exhausted by developing 10 m.<sup>2</sup> of a silver chloride paper, whereas 6 m.<sup>2</sup> of the same paper suffice to exhaust the same amount of developer A. 1-(p-aminophenyl)-3-amino-pyrazoline is produced by refluxing 21.8 grams of 1-(p-acetaminophenyl)-3-aminopyrazoline (F. P. 204° C.) with 220 ml. of 5% aqueous sodium hydroxide solution for 6 hours and thereafter cooling the reaction mass. There are obtained crystals which melt at about 175° C. under decomposition.

**Example 7**

In a hard working developer A of the following composition:

|    |                             |       |  |
|----|-----------------------------|-------|--|
| 70 |                             | Grams |  |
|    | p-Methylaminophenol-sulfate | 2     |  |
|    | Hydroquinone                | 10    |  |
|    | Sodium sulfite              | 40    |  |
|    | Soda                        | 100   |  |
| 75 | Potassium bromide           | 4     |  |

the p-methylaminophenol is replaced by 0.10 gram of the free base 1-(p-aminophenyl)-3-aminopyrazoline or 0.14 gram of the corresponding dihydrochloride (=developer B). Developer B applied for instance to the photographic film "Agfa Printon K" gives a harder gradation than developer A and is of higher capacity.

*Example 8*

A highly active developer A for X-ray films has the 10

|                             | Grams |
|-----------------------------|-------|
| p-Methylaminophenol-sulfate | 3.5   |
| Hydroquinone                | 12    |
| Sodium sulfite              | 15    |
| Sodium carbonate            | 60    |
| Potassium bromide           | 60    |
| Benzotriazole               | 4     |
|                             | 0.05  |

In comparison with this developer A, developer B contains, instead of p-methylaminophenol, only 0.09 gram of 1-(p-aminophenyl)-3-amino-pyrazoline or 0.095 gram of 1-(p-amino-m-methylphenyl)-3-amino-pyrazoline. A comparison of the developing process with Agfa X-ray film shows that developer B has a greater capacity than developer A. The 1-(p-amino-m-methylphenyl)-3-amino-pyrazoline is obtained by refluxing 23.2 grams of 1-(4'-acetylaminomethylphenyl)-3-aminopyrazoline (F. P. 237° C.) with 230 ml. of 10% aqueous sodium hydroxide solution for 12 hours and thereafter cooling the reaction mass. The crystals formed melt at 166° C. under decomposition.

What we claim is:

1. A photographic developing agent which consists essentially of 1-aryl-3-aminopyrazoline, wherein the aryl group is substituted in the 4-position by a radical selected from the group consisting of OH and



wherein R<sub>1</sub> and R<sub>2</sub> are members of the group consisting of hydrogen, alkyl, oxalkyl, sulfoalkyl, and carboxyalkyl, in admixture with a silver halide developing substance comprising a benzene derivative having at least two substituents in the benzene nucleus, said substituents being selected from the group consisting of hydroxy and amino groups and being attached to the benzene nucleus at a position selected from the group consisting of the 1.4 and the 1.2 positions.

2. A photographic developing agent consisting essentially of an alkaline solution of hydroquinone and 1-aryl-3-aminopyrazoline, wherein the aryl group is substituted in the 4-position by a radical selected from the group consisting of OH and



wherein R<sub>1</sub> and R<sub>2</sub> are members of the group consisting of hydrogen, alkyl, oxalkyl, sulfoalkyl, and carboxyalkyl.

3. The developing agent of claim 5 wherein the proportion, by weight, between the hydroquinone and the 1-aryl-3-aminopyrazoline is between about 135 to 1 and about 30 to 1.

4. A developing agent consisting essentially of 1-p-aminophenyl-3-aminopyrazoline and hydroquinone.

5. A developing agent consisting essentially of 1-p-hydroxyphenyl-3-aminopyrazoline and hydroquinone.

6. A silver halide layer in which is incorporated a developing agent consisting essentially of 1-aryl-3-aminopyrazoline wherein the aryl group is substituted in the

4-position by a radical selected from the group consisting of OH and



wherein R<sub>1</sub> and R<sub>2</sub> are members of the group consisting of hydrogen, alkyl, oxalkyl, sulfoalkyl, and carboxyalkyl.

7. A silver halide layer in which is incorporated a developing agent consisting essentially of 1-aryl-3-aminopyrazoline, wherein the aryl group is substituted in the 4-position by a radical selected from the group consisting of OH and



wherein R<sub>1</sub> and R<sub>2</sub> are members of the group consisting of hydrogen, alkyl, oxalkyl, sulfoalkyl, and carboxyalkyl, in admixture with a silver halide developing substance comprising a benzene derivative having at least two substituents in the benzene nucleus, said substituents being selected from the group consisting of hydroxy and amino groups and being attached to the benzene nucleus at a position selected from the group consisting of the 1.4 and the 1.2 positions.

8. A silver halide layer in which is incorporated a developing agent consisting essentially of hydroquinone and 1-aryl-3-aminopyrazoline wherein the aryl group is substituted in the 4-position by a radical selected from the group consisting of OH and



wherein R<sub>1</sub> and R<sub>2</sub> are members of the group consisting of hydrogen, alkyl, oxalkyl, sulfoalkyl, and carboxyalkyl.

9. The process of developing photographic silver halide layers which comprises treating the silver halide layers with a developing agent consisting essentially of an alkaline solution of 1-aryl-3-aminopyrazoline wherein the aryl group is substituted in the 4-position by a radical selected from the group consisting of OH and



wherein R<sub>1</sub> and R<sub>2</sub> are members of the group consisting of hydrogen, alkyl, oxalkyl, sulfoalkyl, and carboxyalkyl.

10. The process of developing photographic silver halide layers which comprises treating the silver halide layers with a developing agent consisting essentially of 1-aryl-3-aminopyrazoline wherein the aryl group is substituted in the 4-position by a radical selected from the group consisting of OH and



wherein R<sub>1</sub> and R<sub>2</sub> are members of the group consisting of hydrogen, alkyl, oxalkyl, sulfoalkyl, and carboxyalkyl in admixture with a silver halide developing substance comprising a benzene derivative having at least two substituents in the benzene nucleus, said substituents being selected from the group consisting of hydroxy and amino groups and being attached to the benzene nucleus at a position selected from the group consisting of the 1.4 and the 1.2 positions.

11. The process of developing photographic silver halide layers which comprises treating the silver halide layers with a developing agent consisting essentially of

an alkaline solution of hydroquinone and 1-aryl-3-amino-pyrazoline wherein the aryl group is substituted in the 4-position by a radical selected from the group consisting of OH and



wherein R<sub>1</sub> and R<sub>2</sub> are members of the group consisting of hydrogen, alkyl, oxalkyl, sulfoalkyl, and carboxyalkyl.

References Cited in the file of this patent

FOREIGN PATENTS

679,678 Great Britain ----- Sept. 24, 1952

UNITED STATES PATENT OFFICE  
CERTIFICATE OF CORRECTION

Patent No. 2,852,374

September 16, 1958

Hans Ulrich et al.

It is hereby certified that error appears in the above numbered patent requiring correction and that the said Letters Patent should read as corrected below.

In the grant, lines 3 to 5, for "assignors to AGFA Aktiengesellschaft für Photofabrikation, of Leverkusen, Germany, a corporation of Germany," read -- assignors to AGFA Aktiengesellschaft, of Leverkusen, Germany, a corporation of Germany, --; line 14 for "AGFA Aktiengesellschaft für Photofabrikation, its successors" read -- AGFA Aktiengesellschaft, its successors --; in the heading to the printed specification, lines 5 to 7, for "assignors to AGFA Aktiengesellschaft für Photofabrikation, Leverkusen, Germany, a corporation of Germany" read -- assignors to AGFA Aktiengesellschaft, Leverkusen, Germany, a corporation of Germany --; column 5, line 17, Example 8, for

Sodium carbonate - - - - 60

read

Sodium carbonate - - - - 40

Signed and sealed this 13th day of January 1959

(SEAL)

Attest:

KARL H. AXLINE  
Attesting Officer

ROBERT C. WATSON  
Commissioner of Patents